



US005254821A

**United States Patent** [19]

Walters

[11] **Patent Number:** 5,254,821[45] **Date of Patent:** Oct. 19, 1993[54] **SELECTIVELY MICROWAVE-PERMEABLE MEMBRANE SUSCEPTOR SYSTEMS**

[75] Inventor: Glenn J. Walters, Duxbury, Mass.

[73] Assignee: Advanced Dielectric Technologies, Inc., Taunton, Mass.

[21] Appl. No.: 641,533

[22] Filed: Jan. 15, 1991

[51] Int. Cl.<sup>5</sup> H05B 6/80

[52] U.S. Cl. 219/10.55 E; 219/10.55 F; 219/10.55 M; 99/DIG. 14; 126/390; 426/107; 426/234; 426/243

[58] Field of Search 219/10.55 E, 10.55 F, 219/10.55 M; 426/107, 234, 113, 243; 99/DIG. 14; 343/18-18 A; 126/390

[56] **References Cited****U.S. PATENT DOCUMENTS**

- 3,302,632 2/1967 Fichtner ..... 219/10.55 E  
 3,887,920 6/1975 Wright et al. ..... 343/18 A  
 4,398,077 8/1983 Freedman et al. ..... 219/10.55 E  
 4,641,005 2/1987 Seiferth ..... 219/10.55 E  
 4,814,568 3/1989 Keefer ..... 219/10.55 E  
 4,831,224 5/1989 Keefer ..... 219/10.55 E  
 4,864,089 9/1989 Tighe et al. ..... 219/10.55 E  
 4,883,936 11/1989 Maynard et al. ..... 219/10.55 F

- 4,888,459 12/1989 Keefer ..... 219/10.55 E  
 4,904,836 2/1990 Turpin et al. ..... 219/10.55 E  
 4,927,991 5/1990 Wendth et al. ..... 219/10.55 F  
 4,962,000 10/1990 Emslander et al. ..... 219/10.55 E  
 4,962,293 10/1990 Lackey ..... 219/10.55 E  
 4,970,360 11/1990 Pescheck et al. ..... 219/10.55 E  
 5,038,009 8/1991 Babbitt ..... 219/10.55 E

**OTHER PUBLICATIONS**

International Search Report PCT/US92/07594.

Primary Examiner—Bruce A. Reynolds

Assistant Examiner—Tu Hoang

Attorney, Agent, or Firm—Douglas R. Wolf

[57]

**ABSTRACT**

A selectively permeable membrane microwave susceptor for use in food packaging is disclosed. The susceptor comprises a substrate having at least one absorbing coating and at least one reflecting coating deposited thereon. Either one or both of the absorbing coating or the reflecting coating can be varied to control the amount of microwave energy reaching the absorbing coating, thereby controlling the overall amount of susceptor heating.

**24 Claims, 6 Drawing Sheets**



Fig. 1 (Prior Art)



Fig. 2



Fig. 3



Fig. 4



Fig. 5



Fig. 6



Fig. 7



Fig. 8



Fig. 9



Fig. 10



Fig. 11



Fig. 12



Fig. 13



Fig. 14

## SELECTIVELY MICROWAVE-PERMEABLE MEMBRANE SUSCEPTOR SYSTEMS

### FIELD OF THE INVENTION

The present invention relates to microwave susceptors for use in packaging of microwaveable food products wherein the susceptor is designed to provide a predetermined reflectivity, transmissivity and absorbance of microwave radiation.

### BACKGROUND OF INVENTION

Microwave ovens are well known devices for quickly and conveniently heating foods. However, microwave cooking is known to be unsatisfactory for a variety of food items, and particularly for food items requiring browning or crisping by surface heating. Microwave cooking relies upon dielectric heating of foods responsive to microwave radiation; thus, the heating characteristics in a microwave oven for some food products are dramatically different from those experienced in a conventional oven. Additionally, the use of microwave ovens can result in undesirable temperature differentials for a variety of food products. For example, some food products, when cooked in a microwave oven, will heat to a greater extent on the interior of the product rather than on the surface as a result of the dielectric microwave heating which favors heating of the product interior. This effect can be contrasted with the results of cooking in a conventional oven in which crisping or browning is achieved by exterior heating of the food item.

Furthermore, an additional problem encountered with microwave cooking is the migration of moisture contained on the interior of the food product. Specifically, in many food products, microwave radiation causes moisture contained on the interior of the food product to migrate to the product surface during cooking. The resulting food product is often left with a soggy surface that is generally undesirable in that it imparts an unsatisfactory texture and taste to the food product.

The above problems are well known in the art of microwave cooking and numerous attempts have been made to solve them. For example, various packages for microwaveable food include susceptors which undergo an increase in temperature in response to microwave radiation. Such microwave susceptors generally comprise a thin metal electrode, usually aluminum, deposited upon the surface of a substrate. The surface resistivity of these susceptors is typically in the range of about 10-500 ohms per square.

The film susceptors described above often suffer performance and physical deterioration when exposed to microwave radiation. This deterioration is a result of very rapid heating which occurs during the early stage of the heating cycle. This heating causes the substrate to undergo dimensional changes which damages the metal electrode on the substrate surface. When this electrode damage and deterioration occurs, these susceptors become less reflective, more transmissive and less absorptive to microwave radiation during heating in the microwave oven and, in so doing, experience dramatic, uncontrolled changes in heating performance. Additionally, such uncontrolled susceptors have raised concerns about chemicals leaching from the substrate or adhesives thereon into the food product, as a result of the high temperatures which occur in the susceptor

during the early stages of the heating cycle. Thus, it would be very desirable to provide susceptors in which microwave power is reflected, transmitted and absorbed in a predetermined combination and which would have better temperature stability, lower temperature performances, and improved consistency in transmission, reflectivity and absorption throughout its exposure to microwave radiation during cooking.

Among the susceptors that are currently used in microwave cooking, a number of other significant problems exist. For example, current susceptors often result in a non-uniform heating of the food product. Such susceptors often produce a food product that is over-heated and overcooked in some regions and under-heated and uncooked in other regions. Such problems are particularly evident in large food items such as pizzas, pies, turnovers and the like.

Furthermore, prior art susceptors generally suffer from a lack of control of temperature of the susceptor itself. In prior art susceptors, the only controllable variables to effect the temperature rise have been the initial resistivity of the susceptor electrode and the substrate material. However, when subjected to microwave radiation, such susceptors are known to undergo physical changes resulting from the heating of the susceptor which causes the substrate to shrink or expand with the result that the metal electrode on the substrate surface is damaged. The damage of the metal electrode layer on the susceptor surface results in a significant decrease in microwave energy absorption and a corresponding increase in susceptor transmission of microwave radiation, thereby resulting in a significant decrease in the heating performance of the susceptor upon the outside of the food product combined with increased induction heating performance resulting from the increase in microwave transmission into the food product.

At least one successful attempt has been made in the prior art to control the damage to the susceptor and to enhance susceptor performance by using the susceptor in combination with a separate, reflecting grid to control the amount of microwave radiation that reaches the susceptor surface. This attempt is described in detail in U.S. Pat. No. 4,927,991 to Wendt, et al. the disclosure of which is incorporated herein by reference. Although addressing a number of significant issues relating to the deficiencies of prior art microwave susceptors, the product described in the Wendt et al. patent suffers by requiring a very costly and complex addition to the microwaveable food package and by creating an inherent arcing possibility at the site of any nicks or sharp edges in such reflecting foil grids.

Thus, a significant need exists for a simple, inexpensive microwave susceptor for use in food packaging that will heat evenly in a predictable manner and will experience no more than minimal deterioration when subjected to microwave radiation during the cooking cycle.

### SUMMARY OF THE INVENTION

The present invention relates to a membrane-type microwave susceptor system comprising a substrate upon which is deposited an absorbing coating or coatings adapted to primarily absorb microwave radiation to generate heat, and a selectively permeable reflecting membrane or coating adapted to reflect a predetermined amount of microwave radiation. The reflecting coating(s) is designed to have known reflectance and

transmittance characteristics for microwave energy, thereby reducing the amount of microwave radiation that contacts the absorbing coating. This results in the ability to control the degree of heating of the susceptor and reduces the likelihood of susceptor failure due to overheating or uncontrollably rapid heating. Thus, by using reflective coatings as microwave energy barriers, susceptor membranes having varying degrees of microwave permeability can be fabricated. Such selectively permeable membranes are characterized by the ability to inherently protect an absorbing coating deposited thereon, or a food product located adjacent to the membrane from excessive microwave energy and inductive heating resulting therefrom, while simultaneously providing a source of conventional, convective or conductive, infrared heating to the food product.

The coatings may be deposited on the same or on opposite sides of the substrate and can comprise the same or different materials. When deposited on opposite sides of the substrate, susceptor deformation and failure is further reduced by providing a susceptor which undergoes a more uniform heating on both sides of the substrate and thereby reduces the likelihood of deformation caused by differential expansion or contraction of the substrate at a localized substrate surface.

Additionally, the present invention eliminates the need to provide a separate grid for controlling the amount of microwave energy that reaches the susceptor surface. The present invention results, rather, in a selectively permeable membrane susceptor system having performance characteristics substantially equal to or better than those of the prior art grid and susceptor combinations.

#### BRIEF DESCRIPTION OF THE DRAWING

FIG. 1 is a graph depicting schematic curves for reflected, transmitted and absorbed microwave energy for a conventional microwave susceptor.

FIG. 2 is a cross-sectional schematic representation of a microwave susceptor having an absorbing film and a reflecting film.

FIG. 3 is a schematic, perspective representation of one embodiment of a microwave susceptor having a discontinuous reflecting film.

FIG. 4 is a schematic, perspective representation of a second embodiment of a microwave susceptor having a discontinuous reflecting film.

FIG. 5 is a schematic, perspective representation of a microwave susceptor having non-uniform heating characteristics.

FIG. 6 is a schematic, perspective representation of a microwave susceptor having multiple absorbing coatings and a single reflecting coating.

FIG. 7 is a schematic, perspective representation of a microwave susceptor having a single absorbing coating and multiple reflecting coatings.

FIG. 8 is a schematic perspective representation of a microwave susceptor having multiple absorbing and reflecting coatings.

FIG. 9 is a graph plotting reflected, absorbed, and transmitted microwave energy as a function of time for a conventional microwave susceptor film.

FIG. 10 is a graph plotting temperature performance as a function of time for a conventional microwave susceptor film.

FIG. 11 is a graph plotting reflected, absorbed, and transmitted microwave energy as a function of time for

a microwave susceptor film comprising one of embodiments of this invention.

FIG. 12 is a graph plotting temperature performance as a function of time for the susceptor film of FIG. 11.

FIG. 13 is a graph plotting reflected, absorbed, and transmitted microwave energy as a function of time for a second embodiment of the microwave susceptor of this invention.

FIG. 14 is a graph plotting temperature performance as a function of time for the microwave susceptor of FIG. 13.

#### DETAILED DESCRIPTION OF THE INVENTION

15 Performance of known susceptors is depicted in FIG. 1, which is a schematic representation of the reflected power, transmitted power and absorbed power for a typical microwave susceptor of the prior art.

Typical prior art susceptors are made by depositing a 20 thin film metal upon a polyester substrate using any of a number of known metal deposition techniques. When exposed to microwave radiation, the metal coating of the susceptor will absorb the radiation and rapidly become relatively hot. This large, rapid heat load can

25 produce dimensional changes in the substrate, such as shrinkage. These dimensional changes often result in cracks or other discontinuities forming in the metal coating and these cracks or discontinuities result in conductivity breaks in the metal film. This process,

30 referred to herein as electrode breakup, is believed to be associated with irreversible changes which occur in the performance characteristics of the susceptor. When such film breakup occurs, the percentage of microwave power which is reflected, transmitted and absorbed

35 changes, generally resulting in an increased transmittance and a corresponding decrease in the absorption of microwave energy by the susceptor. As microwave energy absorption in the susceptor is decreased, heating of the susceptor will decrease and performance of the 40 susceptor as a browning and crisping mechanism for food products will decrease as well.

In a conventional susceptor, a schematic curve for absorbed power for a susceptor is identified by reference numeral 10 in FIG. 1. In the absorbance curve 10

45 depicted in FIG. 1, the percentage of absorbed power peaks at about 0.5 or 50%, for a susceptor having a surface resistivity of approximately 125-175 ohms per square. The transmitted power for such a susceptor will generally follow the schematic curve identified by reference numeral 12 in FIG. 1. Reflected power for the 50 susceptor will generally follow the schematic curve identified with reference numeral 14.

As shown in FIG. 1, microwave absorbance 10 will peak and then decrease to approximately 5-10% of the microwave energy field. This effect is the result of film damage which occurs if the susceptor becomes overheated. As the electrode develops cracks or discontinuities, its absorbance decreases and susceptor heating will undergo a corresponding decrease. The microwave

60 reflectance 12 decreases significantly once film damage occurs. Thus, as discontinuities develop in the film and electrode, more microwave energy passes through the susceptor. The reflectance curve 12 is seen to change significantly at the time of peak absorbance. Reflectance generally will vary from about 30% at the start of the cooking cycle to about 5% following film breakup. The microwave transmittance 14 increases significantly with decreases in absorbance and reflectance. Transmis-

sion will vary from about 20% at the start of the cooking cycle to about 90% following film breakup.

When the absorbance, reflectance and transmittance properties of prior art susceptors change during microwave cooking cycles, such changes generally result in decreased and very different cooking performances of the susceptor. Initially, the susceptor will overheat. This tends to cause film breakup and may result in the volatilization of chemical species from the substrate or adhesives thereon. The volatilization is undesirable in that it may impart chemicals to the food surface which can affect the taste, appearance or fitness of the food product for consumption. The breakup of the metal film layer in a conventional susceptor is known to increase the surface impedance and, in so doing, results in a decreased heating of the susceptor. Thus, it can be seen in FIG. 1 that the percentage of power transmitted through the susceptor increases significantly during the microwave process while the reflected power and absorbed power both significantly decrease resulting in a significant decrease of the heating of the susceptor.

The change in the performance characteristics of the susceptor is undesirable in many applications in which crisping or browning of a microwaveable food product is desired because it increases the amount of dielectric heating in the interior of the food product while decreasing the amount of thermal heating on the food surface. Thus, it would be desirable to have a mechanism for maintaining the susceptor in a state such that the reflected, transmitted and absorbed power characteristics are relatively unchanged and can remain at predetermined levels throughout the microwave cooking cycle. These effects have been achieved by using the inventive susceptors described herein.

As depicted in FIG. 2, one embodiment of the susceptor 20 of the present invention comprises a substrate 22 upon which is deposited a first coating 24 for absorption of microwave radiation and a second coating 26 for reflection of a portion of the microwave radiation to which the susceptor is exposed. By varying the reflectivity of coating 26, a membrane is created which is selectively permeable to microwave energy—i.e., it has the ability to control the amount of microwave energy reaching the absorbing coating 24. In each case, coatings 24 and 26 can be applied by any deposition process, which will not damage the substrate or the deposited coating. In one embodiment, a vapor deposition process which can be any process in which materials are deposited upon substrates from the vapor phase, is preferred. Deposition methods such as chemical and physical vapor deposition (CVD, PVD) which include sputtering, ion plating, electroplating electron beam and resistive or inductive heating are intended to be included herein. It is pointed out that while methods for providing the electrode material in the vapor phase are preferred, the invention is not intended to be limited as such. Rather, any method for applying microwave absorbing and reflecting coatings can be used, provided the method does not damage the substrate upon which the coatings are being deposited during the deposition process.

The absorbing coating 24 preferably has a resistivity in the range of about 30 to about 500 ohms per square. A variety of electrically conductive materials can be used to form the absorbing electrode 24. As such, the absorbing electrode 24 can comprise a coating of a single metal, a metal alloy, a metal oxide, a mixture of metal oxides, a dispersion of conductive metallic or

non-metallic materials in a binder, or any combination of the foregoing. Suitable exemplary metals include aluminum, iron, tin, tungsten, nickel, stainless steel, titanium, magnesium, copper and chromium. Suitable exemplary metal oxides include oxides of aluminum, iron and tin; however, if not electrically conductive, (for example aluminum oxide), they must be used in combination with an electrically conductive material. Suitable exemplary dispersion materials include carbon black, graphite, powdered metals and metal whiskers.

The selectively permeable reflecting coating 26 preferably has a resistivity in the range of about 10 to about 150 ohms per square and as in the case of the absorbing coating 24, can be any of a wide variety of materials including metals or metallic alloys, oxides or mixtures thereof either alone or as a dispersion in a binder. Preferably, the reflecting film 26 comprises a metal having a higher bulk resistivity than elemental aluminum, thereby allowing an electrode layer that is twice as thick for a given resistivity as compared to elemental aluminum. A thicker film for the reflective layer is preferred because in a thicker layer reflection is favored over transmission and also because, surface oxidation as a percentage of overall film thickness becomes smaller as film thickness is increased. By minimizing the relative percentage of film layer oxidation, performance of the reflective coating is more stable.

The substrate 22 preferably comprises an electrical insulator, e.g. a polymeric film, which can be oriented or unoriented. Materials considered to be useful as the substrate 22 include, for example, polyolefins, polyesters, polyamides, polyimides, polysulfones, polyether ketones, cellophanes and various blends of such materials. Other non-conducting substrate materials such as paper and paper laminates, metal oxides, silicates and cellulosics can be used as well. In one embodiment, the substrate 22 comprises a polyester film of the order of approximately 0.25 mil to approximately 2 mil thick. A thickness of approximately 0.5 mil is preferred.

The embodiment of FIG. 2 is particularly well suited for preventing film breakup of the susceptor for two reasons. First, since a significant portion of microwave energy is reflected by the selectively permeable reflecting coating 26, the absorbing coating 24 does not get as hot, and the substrate 22 is less likely to undergo heat-induced deformation or chemical volatilization. Second, since the films are deposited on opposite sides of the substrate they tend to serve to physically impede substrate shrinkage. Thus, the combination of controlled heating effects and physical restraint of the polymeric substrate 22 caused by coating layers 24 and 26 results in an improved susceptor which provides more constant heating characteristics and is less prone to deterioration caused by substrate deformation when exposed to microwave radiation.

In another embodiment of the invention depicted in FIG. 3, the susceptor 30 includes a microwave reflecting film disposed as a series of separate patterns 36, 38 deposited upon a surface of the polymeric substrate 34. The regions 36, 38 can be in the form of a series of parallel stripes, circles or other patterns, or they can be of some other configuration to allow portions of the microwave field to contact directly the polymeric substrate 32, and consequently, the absorbing coating 34, without being reflected by the reflecting coating regions 36, 38. By selecting the particular material of the reflecting coating regions 36, 38, as well as the physical dimensions of the regions such as coating pattern, thickness, width and

pitch, it is possible to control both the degree to which the reflective coating regions 36, 38 will reflect microwave energy and the amount of energy that is transmitted through the polymeric substrate 32 in the spaces 33 between the regions 36, 38 of reflecting material.

In still another embodiment of the invention depicted in FIG. 4, the susceptor 40 includes a microwave reflecting coating comprising separate regions 46, 48 of reflecting coating applied directly to the surface of the absorbing electrode coating 44 once the absorbing electrode has been deposited upon a surface of the polymeric substrate 42. In this embodiment, regions of the reflecting coating 46, 48 are deposited directly upon the microwave absorbing coating 44 in a manner such that spaces 43 of the absorbing coating 44 are exposed in the areas between the reflecting regions 46 and 48. As before, by selecting a specific material, thickness, width and pitch of the reflecting regions, the amount of the field of the microwave field that is reflected relative the amount of the field that is transmitted can be highly controlled.

Alternatively, the embodiment of the invention depicted in FIG. 4 can be fabricated by a process in which a relatively thick reflective coating is deposited upon one surface of the substrate and then selectively and partially removed using any of a variety of removal techniques to remove portions of the reflective coating. The coating removal can be either complete of (i.e. down to the substrate surface), or partial (i.e. removing only a partial thickness of the reflective coating). If a complete removal technique is used, the resulting substrate will have a patterned reflective coating deposited thereon. On the other hand, if a partial removal process is used, the resulting substrate will have a reflective coating thereon having regions that are relatively thick to reflect microwave energy as well as regions that are relatively thin to absorb microwave energy. This embodiment provides performance characteristics that are similar to those of the dual-coating susceptor in which both the absorbing and the reflecting coating are deposited upon the same side of the substrate.

Additionally, although the embodiment depicted in FIG. 4 does not include material deposited on opposite sides of the polymeric substrate to support the substrate and prevent deformation thereof during microwave heating, the reflective regions serve to limit the amount of microwave energy reaching the absorbing film and thereby prevent the film from overheating and deforming the polymeric substrate or causing volatilization thereof. Thus, susceptor performance is more constant and predictable throughout the cooking cycle.

Although, in each of the embodiments described above, the absorbing coating is a continuous, uniform layer, the present invention is not intended to be limited as such. Rather, the present invention is intended to include susceptors in which either one or both of the absorbing coating and the reflecting coating are provided with a pattern. Accordingly, as with the reflecting layer, the absorbing coating can comprise a series of parallel stripes, circles or other geometric configurations. The pattern of either one or both of the reflecting coating and the absorbing coating can be formed during deposition, or alternatively, the coating can be deposited as a uniform layer with pattern formation occurring during subsequent demetalization steps. Thus, the invention is intended to comprise a susceptor in which the heating performance can be controlled by controlling, among other variables, coating thickness, coating pat-

tern and coating material for both the absorbing coating and the reflecting coating, regardless of whether the two coatings are on the same or opposing sides of the substrate.

In still another embodiment of the invention, both the reflecting and absorbing regions can be designed to have different reflective and absorptive characteristics in different portions of the susceptor. In so doing, different regions of the absorbing layer will receive differing amounts of microwave energy and will, accordingly, heat to different levels. As such, a susceptor of this type is well suited for applications in which it is desired to brown or to crisp different portions of a packaged food product to differing degrees.

One such susceptor is depicted in FIG. 5. In FIG. 5, the susceptor 50 comprises a polymeric substrate 52 having a microwave absorbing coating 54 deposited on one surface thereof. A microwave reflecting coating comprising a plurality of separate, reflecting regions 56, 58, 66, 68, 76, 78 is deposited on the surface of the substrate opposing the surface on which the absorbing film 54 is deposited. In this example, three different zones of reflecting film have been deposited on the substrate to provide three non-uniform heating zones 55, 65, 75 on the susceptor.

A first heating zone 75 is created by depositing large reflecting coating regions 76 and 78 which cover a large surface portion of the substrate. These large regions 76, 78 serve to reflect a large portion of microwave energy and therefore allow a relatively small amount of energy to be absorbed in the absorbing coating 54 in the film portion opposite these large reflecting regions. As such, the susceptor portion having large reflecting regions 76 and 78 will undergo the least amount of heating, and food items positioned adjacent this zone 75 of the susceptor will be subjected to the least amount of browning or crisping.

A second heating zone 65 is created by reflecting regions 66 and 68 which cover a relatively small portion of the substrate area in which such regions are deposited. These small regions 66, 68 serve to reflect only a small portion of microwave energy and therefore allow a relatively large amount of energy to be absorbed in the absorbing electrode coating 54 in the film portion opposite these small reflecting regions. As such, the susceptor portion having small reflecting regions 66 and 68 will undergo the greatest amount of heating. Food items positioned adjacent this zone 65 of the susceptor will be subjected to the greatest amount of browning or crisping.

Finally, a third heating zone 55 is created by reflecting regions 56 and 58 which are of an intermediate size between the large reflecting portions 76 and 78 and the small reflecting portions 66 and 68. Accordingly, food items positioned adjacent to the susceptor in heating zone 55 will undergo an amount of browning or crisping that is between that produced by zones 76 and 66. For example, a susceptor of this type could be used in a frozen dinner having a three different food types to heat each food type to a particular degree. Thus, susceptor heating zone 66 could be positioned in the region over a serving of fried potatoes, thereby allowing the potato surface to be deeply browned; heating zone 75 could be positioned over a serving of vegetables to allow only light cooking thereof; and heating zone 55 could be positioned over a serving of meat to allow an intermediate heating and browning of that serving.

As set forth previously, the differing heating characteristics can be achieved by varying the absorbing layer instead of, or in combination with, providing variations in the reflecting layer. Thus, by patterning the absorbing layer differently in differing heating zones, a non-uniform susceptor heating characteristic can be achieved.

In another embodiment of the invention, the differing heating zones can have a circular configuration. Thus, for example, if it were desired to brown an annular region of a food item, such as the crust of a pizza, the susceptor could be configured to have a center portion that absorbs a higher portion of microwave energy than an annular portion of the susceptor surrounding the center. This configuration would allow a greater percentage of microwave energy to reach the absorbing coating in the annular region, thereby allowing greater heating of the center portion of the susceptor and providing a higher browning heat to the center portion of the pizza.

It is noted that the above, non-uniform susceptors are not intended to be limited strictly to the embodiments described above. Rather, any number of separate heating zones can be created on the susceptor. Furthermore, the differing heating zones can be created by altering any of the variables discussed herein. Thus, each selectively permeable membrane coating could be of the same dimensions, but of materials having different reflective properties. Alternatively, the reflecting films could be of the same material but could be deposited to have different patterns thicknesses, widths or pitches. Additionally, as set forth in the embodiment of FIG. 4, the different reflecting coating portions could be deposited directly upon the surface of the absorbing coating.

The invention is not intended to be limited solely to a susceptor having a single absorbing coating and a single, selectively permeable reflecting coating. Rather the inventive susceptor is intended to include systems having multiple absorbing and/or reflecting coatings. Thus, the invention will include a susceptor having an absorbing coating on both sides of the substrate with a single reflecting layer on one absorbing coating, a susceptor having an absorbing coating on one side of the substrate with reflecting coatings covering both the absorbing coating and the opposing side of the substrate, and a susceptor having both an absorbing coating and a reflecting coating on each side of the substrate.

For example, FIG. 6 depicts a susceptor 80 having a substrate 82 upon which are deposited absorbing coatings 84, 86 on opposing sides of the substrate. A selectively permeable reflecting coating 88 is deposited on absorbing coating 84. In this embodiment a pattern comprising a plurality of circular cutouts 90 has been provided on the reflecting coating 88.

FIG. 7 depicts a susceptor 92 having a substrate 94 upon which is deposited an absorbing coating 96 as well as two selectively permeable reflecting coatings 98, 100. Coating 100 has been patterned by providing a plurality of triangular cutouts 102. Reflecting coating 98 may be patterned, if at all, in a similar or different manner.

FIG. 8 depicts a susceptor 104 having a substrate 106 upon which are deposited two absorbing coatings 108, 110 and two selectively permeable reflecting coatings 112, 114.

## EXAMPLES

## Example 1

In this example, a standard susceptor film was fabricated using a polyester substrate having a thickness of 0.5 mil. Aluminum was coated on one side of the polyester substrate to have an optical density of approximately 0.25 with a resulting surface energy of approximately 75 ohms per square. The susceptor was placed in a microwave test fixture operated at 150 watts and exposed to microwave energy for one minute. FIG. 9 depicts the power fractions of reflected, absorbed, and transmitted microwave energy as a function of time. As can be seen in FIG. 9, the properties of the susceptor begin to change almost immediately, and undergo a continuing change for approximately 20 seconds. Thus, whereas initially the susceptor has a transmissivity of approximately 4%, a reflectivity of approximately 66% and an absorbance of approximately 30%, as the susceptor undergoes breakdown, approximately 25% of the energy is reflected, approximately 25% of the energy is absorbed and approximately 50% of the energy is transmitted through the susceptor.

The result of this susceptor breakdown can be seen in FIG. 10 in which film temperature in two different regions is plotted as a function of time. In each case, the temperature probes were located on the susceptor film with a separation of approximately one inch. At the beginning of the cooking cycle the susceptor film surface is at a temperature of approximately 75° F. and then rises over the first 20 seconds of the cooking cycle to a temperature of approximately 350° F.

## Example 2

In this example, a modified susceptor film having high, constant reflectivity was fabricated. Specifically, a polyester substrate having a thickness of 0.5 mil was coated on one side with an absorbing aluminum coating to an optical density of approximately 0.25. As before, this corresponds to a bulk resistivity or surface energy of approximately 75 ohms per square. The opposite side of the substrate was coated with a pattern which comprised metal stripes of aluminum that were approximately 0.875 inches wide with a spacing between the stripes of approximately 0.2 inches. The stripes were deposited to have a bulk resistivity of approximately 25 ohms per square.

FIG. 11 depicts the power fraction of reflected, absorbed and transmitted microwave energy as a function of time as the susceptor is exposed to microwave energy in a microwave test fixture operated at 150 watts. As can be seen in FIG. 11, the transmitted power of microwave energy using the modified susceptor stays at approximately 0% throughout the heating cycle. The absorbed energy varies from approximately 8% at the beginning of the cycle to approximately 10% at the end of the cycle. Finally, the reflected energy varies from approximately 92% at the beginning of the cycle to approximately 90% at the end of the cycle. Thus, it can be seen that the use of a reflecting coating in connection with the absorbing coating for a microwave susceptor results in a susceptor having reflection, absorption and transmission characteristics that are much more stable and uniform when subjected to microwave energy.

FIG. 12 depicts a plot of temperature as a function of time for this modified susceptor film. As can be seen in FIG. 12, the substrate temperature undergoes a continu-

ous rise in temperature over the heating cycle of the film. The curve shows two test points taken on the susceptor film surface. However, since both test points were located at similar temperature positions during the test, the resulting heating curves are substantially identical. As can be seen in FIG. 12, initially, the susceptor starts at a temperature of approximately 75° F., rises steadily to a temperature approximately 250° F. during the first 15 seconds of microwave exposure and then continues with a gradual rise to approximately 350° F. 10 over the remaining 45 seconds of the test.

### Example 3

In this example, a susceptor very similar to the susceptor of the previous example was fabricated. The 15 only difference was in the width of the stripes of the reflecting coating. Whereas in the previous example the stripes had a thickness of approximately 0.875 inches, in this example, the reflecting stripes each had a width of approximately 0.27 inches. As before, the separation 20 between the stripes was approximately 0.2 inches. As can be seen in FIG. 13, a plot of power fraction versus time, even the use of thin reflecting stripes will dramatically alter the power fraction curves for reflected, 25 absorbed and transmitted microwave energy as compared to those curves for a conventional microwave susceptor. Thus, as shown in FIG. 13, the portion of microwave energy that is transmitted using this susceptor starts at approximately 10%, rises to approximately 40% over the first 15 seconds of microwave exposure and then gradually rises to approximately 15% over the final 45 seconds of the test. Likewise, at the beginning of the test approximately 25% of the microwave energy is absorbed and this gradually falls off to approximately 15% over the test cycle. Finally, at the start of the test, 30 approximately 65% of the microwave energy is transmitted. This falls off to approximately 40% in the first 15 seconds of the test and then gradually to approximately 35% over the remaining 45 seconds of the test.

FIG. 14 depicts temperatures as a function of time for 40 the above susceptor as plotted at two different locations on the susceptor film. On curve number 1, which represents the temperature of the susceptor film in a location lying beneath a reflecting stripe, the susceptor temperature starts at approximately 75° F., rises to approximately 225° F. during the first 20 seconds of microwave exposure and then gradually rises to approximately 250° F. over the remaining 40 seconds of the test. In contrast, 45 curve number 2, representative of the temperature of the susceptor in a section which is not covered by a stripe, also begins at approximately 75° F., rises to approximately 375° F. in the first 20 seconds of the test, and then gradually rises to a final temperature of approximately 400° F. in the remaining period of the test.

Thus, as can be seen from FIG. 14, the use of a microwave susceptor having a patterned reflecting coating provides a susceptor that has differing and controllable temperature characteristics in differing regions of the susceptor.

### EQUIVALENTS

Although the specific features of the invention are shown in some drawings and not in others, this is for convenience only, as each feature may be combined with any or all of the other features in accordance with the invention.

It should be understood however that the foregoing description of the invention is intended merely to be

illustrative thereof, that the illustrative embodiments are presented by way of example only, and that other modifications, embodiments, and equivalents may be apparent to those skilled in the art without departing from its spirit.

Having thus described the invention, what we desire to claim and secure by Letters Patent is:

1. A microwave susceptor for use in food packaging, the susceptor comprising:
  - (a) at least one substrate that is substantially transparent to microwave energy, the substrate having opposed surfaces;
  - (b) at least one microwave-absorptive coating disposed as a pattern upon a portion of one surface of the substrate, said at least one microwave-absorptive coating comprising a plurality of separate, electrically conductive regions; and
  - (c) at least one microwave-reflective coating disposed as a pattern overlapping said at least one microwave-absorptive coating to thereby modify the amount of microwave energy that reaches the microwave-absorptive coating when the susceptor is exposed to a microwave energy field, said microwave-reflective coating comprising a plurality of separate, electrically conductive regions.
2. A microwave susceptor as in claim 1 wherein the substrate has one microwave-absorptive coating and one microwave-reflective coating disposed on opposing sides thereof.
3. A microwave susceptor as in claim 1 wherein a microwave-reflective coating is disposed directly upon a microwave-absorptive coating.
4. A microwave susceptor as in claim 1 wherein the microwave-absorptive coating has a resistivity of between about 30 and about 500 ohms per square.
5. A microwave susceptor as in claim 1 wherein the microwave-reflective coating has a resistivity of between about 10 and about 150 ohms per square.
6. A microwave susceptor as in claim 1 wherein the microwave-absorptive coating comprises a metal and metallic alloy.
7. A microwave susceptor as in claim 6 wherein the microwave-absorptive coating comprises elemental aluminum.
8. A microwave susceptor as in claim 1 wherein the microwave-reflective coating comprises a metal and metallic alloy.
9. A microwave susceptor as in claim 8 wherein the microwave-reflective coating comprises a metal and metallic alloy having a bulk resistivity higher than that of elemental aluminum.
10. A microwave susceptor as in claim 1 adapted to undergo non-uniform heating in the presence of a uniform microwave energy field.
11. A microwave susceptor as in claim 10 wherein the microwave-reflective coating includes a plurality of regions having differing reflectivities.
12. A microwave susceptor as in claim 11 wherein the regions having differing reflectivities comprise microwave-reflective coatings comprising differing materials.
13. A microwave susceptor as in claim 11 wherein the regions having differing reflectivities comprise microwave-reflective coatings having differing patterning geometries.
14. A microwave susceptor as in claim 10 wherein the microwave-absorptive coating includes a plurality of

regions having differing microwave energy absorption characteristics.

15. A microwave susceptor as in claim 14 wherein the regions having differing microwave absorption characteristics comprise microwave-absorptive coatings comprising differing materials. 5

16. A microwave susceptor as in claim 14 wherein the regions having differing microwave absorption characteristics comprise microwave-absorptive coatings having differing patterning geometries. 10

17. A microwave susceptor as in claim 1 having microwave-absorptive coatings disposed on opposing sides of the substrate. 15

18. A microwave susceptor as in claim 1 having microwave-reflective coatings disposed on opposing sides of the substrate. 20

19. A microwave susceptor as in claim 17 having microwave-reflective coatings disposed upon each of 25 the microwave-absorptive coatings.

20. A microwave susceptor as in claim 1 comprising a substrate and a microwave-reflective coating disposed thereon, the coating being at least partially removed in a pattern to provide microwave-absorptive characteristics in regions where the coating has been removed.

21. A microwave susceptor for use in food packaging, the susceptor comprising:

a substrate that is substantially transparent to microwave energy; 30

at least two microwave-absorptive coating regions deposited as a pattern on at least one surface of the substrate, said microwave-absorptive coating regions capable of producing heat when exposed to microwaves and having a resistivity of about 75 ohms per square; and

at least two microwave-reflective coating regions having a resistivity of about 10 ohms per square, said microwave reflective coating regions deposited as a pattern overlapping said microwave-absorptive coating regions.

22. A microwave susceptor for use in food packaging, the susceptor comprising:

- (a) a substrate that is electrically non-conductive;
- (b) at least one microwave-absorptive, electrically conductive electrode disposed upon at least a portion of a surface of the substrate; and
- (c) a plurality of microwave-reflective, electrically conductive electrodes disposed overlapping said microwave-absorptive electrode as a plurality of electrically conductive regions.

23. The susceptor of claim 22, wherein said microwave-absorptive electrode comprises separate, electrically conductive regions, each region electrically conductive within said region and electrically isolated from other said separate regions. 25

24. The susceptor of claim 22, wherein said microwave-reflective electrodes are separated from each other by an electrically non-conductive gap.

\* \* \* \* \*

35

40

45

50

55

60

65